

Nov. 29, 1927.

1,650,951

H. D. MATTHEWS

THERMOSTATIC MATERIAL

Filed March 18, 1925



WITNESSES:

Carl J. Loesch  
H. M. Biebel

INVENTOR  
Howard D. Matthews

BY  
Wesley G. Barr  
ATTORNEY

## UNITED STATES PATENT OFFICE.

HOWARD D. MATTHEWS, OF EDGEWOOD, PENNSYLVANIA, ASSIGNOR TO WESTINGHOUSE ELECTRIC & MANUFACTURING COMPANY, A CORPORATION OF PENNSYLVANIA.

## THERMOSTATIC MATERIAL.

Application filed March 18, 1925. Serial No. 16,341.

My invention relates to temperature controlled devices and particularly to thermostatic material and bimetallic thermostats.

One object of my invention is to provide 5 a bimetallic thermostat, the elements of which shall have different temperature coefficients and that shall be composed of material capable of being subjected to relatively high temperatures without substantial 10 change of structure after repeated operations thereof.

In practicing my invention, I provide a bimetallic thermostatic element comprising two metallic elements, one of said elements 15 being a chromium steel.

The single figure of the accompanying drawing illustrates two curves showing the relative temperature coefficients of expansion of two metals employed in practicing my 20 invention.

The use of two more or less closely united strips of metal to form a bimetallic thermostatic member that is responsive to heat has long been known. Iron and brass have usually 25 been employed for such purposes and will function properly if the temperatures to which they are subjected do not exceed a relatively limited value. However, when it is desired to operate at relatively high 30 temperatures, such as from 200° to 500° or 600° C. the above named metals rapidly lose their original elasticity and the device fails to function properly.

I have found that a thermostatic member 35 comprising two metal elements, one of these being a chromium steel, and used in connection with a copper-nickel alloy, generally known as Monel metal, will function properly at very much higher temperatures than has been heretofore thought possible.

The curve 11 shows the temperature coefficients of expansion of a copper-nickel alloy, comprising substantially two-thirds copper and one-third nickel and generally known as 45 Monel metal, between the temperature range of zero to 550° C. While the curve is illustrated as being substantially a straight line, values may vary slightly therefrom, but the curve shows substantially correct 50 values.

The second member of such bimetallic heat-responsive device is a chromium steel comprising substantially 10 to 15% of chromium with admixtures of phosphorus, sili-

con, manganese, carbon and sulphur, the latter being present in relatively small amounts only. Curve 12 illustrates the temperature coefficients of expansion of such chromium steel alloy up to temperatures of about 550° C. and it may be noted that the difference 60 between the respective temperature coefficients of expansion varies but little over the entire range of temperature. Such a chromium steel is not a reversible alloy but the transformation points thereof occur at temperatures above 750° C. In some samples that have been tested, these transformation points occur at about 850° C. to 950° C. Hence, it is necessary that a bimetallic heat-responsive device built according to my invention, be used at temperatures well below those at which the transformations take place.

The chromium steel may be suitably heat treated after being made a part of a finished 75 device to be tempered, thereby permitting of obtaining a heat-responsive device having a permanent and relatively high elasticity that will continue substantially constant even though subjected to repeated temperature changes of relatively large amount.

Any desired construction of the heat-responsive device may be employed, that is, the two strips or plates may be welded over the entire abutting surfaces or they may be secured at their respective ends only, either 80 by welding or riveting, and any suitable or desired construction is within the scope of my invention, which comprises more particularly the use of a chromium steel alloy having 85 an appreciable admixture of chromium whose transformation points occur above a temperature of 750° C.

Various modifications and changes may be made without departing from the spirit 95 of the invention, and I desire therefore, that only such limitations shall be placed thereon as are imposed by the prior art.

I claim as my invention:

1. A heat responsive device consisting of 100 two metallic elements, one of said elements being an irreversible chromium steel alloy, and the other element being an alloy of copper and nickel.

2. A heat responsive device consisting of 105 two metallic elements, one of said elements being an irreversible chromium steel alloy, whose transformation points occur at tem-

peratures above 750° C., and the other element being a copper nickel alloy containing not over 67% of copper.

3. A heat responsive device consisting of two metallic elements, one of said elements being steel containing not over 15% of chromium, and the other of said elements being

a copper nickel alloy containing not over 67% of copper.

In testimony whereof, I have hereunto 10  
subscribed my name this 11 day of March,  
1925.

HOWARD D. MATTHEWS.